

## UNITED STATES PATENT OFFICE

2,025,989

METHOD FOR SOAKING NATURAL  
SILK FIBERS

Philip Kaplan, Brooklyn, N. Y.

No Drawing. Application August 31, 1933.  
Serial No. 687,582

5 Claims. (Cl. 28—1)

This invention relates to a method and a product for soaking natural silk fibers. It is customary to soak silk fibers prior to throwing or twisting and winding. This soaking is for the purpose of softening the fibers so that they may be handled. It is particularly desirable that this soaking be not of such a nature as to remove the gum which surrounds the fiber, in fact, one of the objects of this invention is to produce a soaking material or bath that will prevent degumming and particularly during the later manipulation of the silk, as degumming tends to interrupt subsequent operations and may clog the machinery to a disastrous extent as will be later described.

The materials used for the purpose of soaking natural silk fibers generally consist of soap and raw oils such as olive oil, neat's-foot oil and in some instances, mineral oil or of prepared emulsified oils consisting of various emulsifying agents in combination with the oils as above set forth.

In order to impart hygroscopicity to the silk, it has been customary to use, in conjunction with the above mentioned compounds, glycerine, or diethylene glycol.

The use of the above mentioned compounds are fraught with certain limitations which may be the source of considerable trouble in the subsequent steps of preparing the yarn or knitting or weaving, for instance, when soap and raw oil mixtures are used, considerable degumming usually results. This is particularly noticeable if the soap and oil mixtures are carelessly prepared. If this stripping takes place in the winding or in the knitting operations, the needles become clogged.

In making such products as emulsions for this purpose, it is often found necessary to have a considerable percentage of fatty acids present. The presence of fatty acids is objectionable in that the needles of the machines become corroded, which results in a roughening of the fibers or increases stripping or both. To neutralize these free fatty acids great care must be taken in introducing the proper type and amount of alkali, otherwise the degumming will be increased and there are other disadvantages in the use of these compounds which produce tenderness and/or stickiness which in turn result in mechanical difficulties in the operation of knitting or weaving and which may also result in sleaziness and mildew, both of which are exceedingly objectionable.

The particular advantages to be found in the use of the product and method which I am about

to describe are that it is unnecessary to add alkali, glycerine, mineral oils, raw oils or soap.

The ease with which my material boils off makes it unnecessary to resort to high temperatures or the use of excess soaps which are found necessary to boil off mineral oil and raw oils and thus preventing degumming.

Because of the high penetration power, hygroscopic silk is obtained by the use of my material alone.

The products that I use to obtain the desired results are such as are obtained by sulphonating tallow, palm oil, waxes, olive oil, castor oil and fatty alcohols to such an extent that the organically combined  $SO_3$  will be high, and I prefer and desire that the organically combined  $SO_3$  be not less than 5% but may be as high as 12%. By this process, extremely soluble and highly penetrating fatty compounds are obtained and the fatty acids derived therefrom are of particularly high "titre" or solidifying point, even though the oil treated by that process is originally in a fluid state and while I may use any of the materials therein described, I particularly choose for this purpose those compounds described as tallow, palm oil, waxes, olive oil, castor oil and fatty alcohols.

I have found that the desired materials treated and sulphonated in the manner set forth have the characteristic of being absorbed chemically by the natural silk fibers and it is to this characteristic that I attribute certain important advantages to be derived from their use, this in contradistinction to the compounds heretofore used which depend upon their rather individual physical properties.

As an example of the method employed in using the products herein described, I take 60 pints of the fatty materials sulphonated to from 5 to 12% organically combined  $SO_3$  based upon the fatty content thereof, as above referred to, and dissolve this fatty material in 60 gallons of water at a temperature of 85° F. Into this bath I immerse 100 lbs. of silk yarn for a period of about 12 hours. At the time of this treatment the silk is probably in standard commercial skeins and after the period of soaking, the skeins are removed from the bath and placed in a hydro-extractor where the moisture is removed to the desired extent. Thereafter the silk is handled or manipulated in the usual manner and by the practices common in the art. This method and material produces a silk yarn which has all of the advantages and none of the disadvantages heretofore referred to.

The foregoing example assumes the treatment of Japanese silk, but as silk fibers vary, dependent upon their origin, so the material and treatment will be varied, for example with China, Italian or Tussah silks; the proportion of the fatty compound used and the time and temperature will be varied as final results will dictate, but such variations as are required may be made without departing from the spirit of this invention.

5 10 Having carefully and fully described my invention, what I claim and desire to obtain is:

11 15 1. The process of treating natural silk fibers which consists of soaking the fibers in a bath containing high titre fats which have been sulphonated to a minimum of 5% organically combined SO<sub>3</sub> based on the fatty content.

16 20 2. The method of treating natural silk fibers which consists of soaking fibers in a bath containing a sulphonated tallow which has been sulphonated to at least 5% organically combined

SO<sub>3</sub> based on the fatty content of said material.

3. The method herein described for treating natural silk fibers which consists of soaking the fibers for approximately 12 hours in a bath containing sulphonated castor oil containing at least 12% organically combined SO<sub>3</sub> based on the fatty content.

4. The method herein described of treating natural silk fibers which consists of soaking the fibers for approximately 12 hours in a bath containing a fatty material sulphonated to contain at least 12% organically combined SO<sub>3</sub> based on the fatty content.

5. The method herein described of treating natural silk fibers which consists of soaking the fibers for approximately 12 hours in a bath containing olive oil sulphonated to a minimum of 12% organically combined SO<sub>3</sub> based on the fatty content.

PHILIP KAPLAN. 20